

No. 753,982.

PATENTED MAR. 8, 1904.

S. R. HOLLAND.

PREPARED ROOFING,

APPLICATION FILED JUNE 23, 1903.

NO MODEL.



Fig. 2.



Witnesses  
Alfred A. Kier  
Malvina.

Emmetor  
Stanley R. Holland  
by Higdon & Oongan & Hopkins attys.

## UNITED STATES PATENT OFFICE.

STANLEY R. HOLLAND, OF ST. LOUIS, MISSOURI.

## PREPARED ROOFING.

SPECIFICATION forming part of Letters Patent No. 753,982, dated March 8, 1904.

Application filed June 23, 1903. Serial No. 162,739. (No specimens.)

*To all whom it may concern:*

Be it known that I, STANLEY R. HOLLAND, a citizen of the United States, and a resident of St. Louis, State of Missouri, have invented 5 certain new and useful Improvements in Prepared Roofing, of which the following is a specification containing a full, clear, and exact description, reference being had to the accompanying drawings, forming a part hereof.

10 This invention relates to improvements in prepared roofing; and it consists in the novel construction, arrangement, and combination of parts, as will be fully hereinafter described and claimed.

15 The object of this invention is to provide a prepared roofing constructed of various materials and coated on its outer surface with crushed shell.

In the drawings, Figure 1 is a perspective view of a roll of my improved prepared roofing, a corner thereof being separated to show the various layers. Fig. 2 is a detailed enlarged sectional view of a portion of the roofing material.

25 The prepared roofing consists, first, of a heavy layer of felt 3, saturated with asphalt. 4 indicates a coating of genuine Trinidad asphalt, and 5 a layer of buckram or burlap saturated with asphalt.

30 6 indicates a coating of genuine Trinidad asphalt, and 7 represents crushed shell spread over the entire surface of the material and adheres thereto by means of the asphalt coating.

The one edge 8 of the material is provided 35 with a margin, say, about two inches in width, which is sprinkled with a coating of marble-dust 9. This is for the purpose of providing a perfect water-tight joint when the material is placed in proper position upon the roof and

properly overlapped, bringing the end or felt 40 surface over the margin.

The material is constructed in long sheets and when finished rolled, as indicated in Fig. 1.

The essential feature of my invention is the manner of coating the material with crushed 45 shell, the purpose of which making a neater, more even, and white roof, the shell retaining its color, whereas a material such as gravel and sand loses its natural color by being exposed to the weather and giving a dirty appearance to the roof. By the use of the marble-dust margin a more perfect joint can be made.

What I claim is—

1. A material for prepared roofing composed 55 of layers of felt, burlap and asphalt adhesively retained together, the outer surface being covered with crushed shell, a margin formed on the one edge of the material and sprinkled with marble-dust, substantially as specified. 60

2. A material for prepared roofing composed of a layer of felt, asphalt placed on the layer of felt, a layer of burlap located on the asphalt, asphalt placed on the upper surface of the layer of burlap, crushed shell sprinkled 65 on the asphalt and adhesively retained in a perfect flat position upon the surface of the roofing material, a margin formed on the one edge of the material, said margin sprinkled with marble-dust, substantially as specified. 70

In testimony whereof I have signed my name to this specification in presence of two subscribing witnesses.

STANLEY R. HOLLAND.

Witnesses:

ALFRED A. EICKS,  
JOHN C. HIGDON.